

Patented Nov. 1, 1927.

1,647,301

# UNITED STATES PATENT OFFICE.

KURT K. LEDIG, OF NEWARK, NEW JERSEY, ASSIGNOR TO AMERICAN PLATINUM WORKS, OF NEWARK, NEW JERSEY, A CORPORATION OF NEW JERSEY.

## ALLOY FOR PEN POINTS.

No Drawing.

Application filed March 1, 1926. Serial No. 91,621.

This invention relates to metallic alloys of a particularly hard, tough, noncorrodible nature, adapted specifically for use on the points of writing pens of the highest type.

It is one of the features of the invention to provide an alloy that may be substituted for osmium iridium, as commonly used for gold pen points, and which possesses superior characteristics, such for instance as greater uniformity in grain, color and uniting properties to pen nibs.

These objects are accomplished by the novel combination and blending of certain rare or noble metals as hereinafter described and later claimed.

The preferred form of the alloy is composed of molybdenum predominately, together with lesser amount of other metals selectively of the platinum group, said group consisting of platinum, iridium, palladium, rhodium, osmium, and ruthenium, in the approximate proportions set forth:

|                          | Parts. |
|--------------------------|--------|
| Molybdenum               | 80     |
| Metals of platinum group | 20     |

I have found that the proportions of molybdenum may be reduced and nickel or a nickel copper alloy added, and lesser portions of other metals selectively of the platinum group, said group consisting of platinum, iridium, palladium, rhodium, osmium, and ruthenium, this nickel-copper alloy containing a large percentage of nickel, and some copper which tends to render the alloy more easily workable.

The properties of this last example of the alloy may be given as follows:

|                      | Parts. |
|----------------------|--------|
| Molybdenum           | 60     |
| Nickel-copper alloy  | 30     |
| Rhodium or ruthenium | 10     |

I have found that the proportions of the nickel or nickel-copper alloy may be reduced and tungsten added in small amounts, which will produce an alloy possessing great strength and having the properties above set forth. The properties of this last example of the alloy may be given as follows:

|                      | Parts. |
|----------------------|--------|
| Molybdenum           | 60     |
| Nickel-copper alloy  | 20     |
| Tungsten             | 10     |
| Rhodium or ruthenium | 10     |

I have also found that 60 parts molyb-

denum and 30 parts nickel-copper alloy or 30 parts of nickel alone with 6 parts platinum and 4 parts osmi-iridium will produce an alloy having the properties above set forth.

In some cases, I have also found, by reducing the nickel or nickel-copper alloy to 20 parts and adding 60 parts molybdenum, 10 parts tungsten, 6 parts platinum, and 4 parts osmi-iridium, an alloy possessing great strength and having the properties above set forth will be produced.

In the detail description I have set forth several different forms of my invention all of which possess in some degree the characteristics heretofore set forth, which in others some of the properties are more pronounced; and while the proportions of the ingredients of the alloy generally may be varied between fairly wide limits to meet the conditions and requirements of the several uses to which the alloy may be put, yet the general properties above set forth are present in some degree in each of the forms specified.

The foregoing is considerably lower in specific gravity than osmium iridium and lacks its characteristic brittleness, being relatively tough, dense and hard. It is furthermore readily fused with gold, presenting a silver-gray color, capable of receiving a high polish.

It will be obvious to those skilled in the art, after understanding my invention, that modifications and substitutions of equivalents may be made in the alloy without departing from the spirit and scope of my invention, and that my invention is not to be limited to any particular method of making the alloy, and I aim in the appended claims to cover all modifications, substitutions and changes within the scope of my invention.

Having thus described my invention, what I claim as new and desire to secure by Letters Patent, is:

1. An alloy of the class described, consisting predominately of molybdenum and the balance principally of nickel and copper, the nickel exceeding the copper, and lesser amounts of tungsten and other metals selectively of the platinum group, said group consisting of platinum, iridium, palladium, rhodium, osmium and ruthenium.

2. An alloy of the class described containing sixty parts molybdenum, twenty parts

nickel-copper alloy said alloy consisting of 70 parts nickel and 30 parts copper, ten parts tungsten, and ten parts ruthenium.

3. An alloy of the class described, non-fibrous and of extreme hardness, said alloy containing sixty parts molybdenum, twenty parts nickel-copper alloy said alloy consisting of seventy parts nickel and thirty parts

copper, ten parts tungsten, and ten parts of other metals selectively of the platinum group, said group consisting of platinum, iridium, palladium, rhodium, osmium, and ruthenium.

This specification signed and witnessed this 25th day of February, 1926.

KURT K. LEDIG.